

Aug. 28, 1951

G. E. FALLESEN ET AL

2,566,180

DIRECT POSITIVE PHOTOGRAPHIC COLOR PROCESS

Filed Aug. 13, 1948



GEORGE E. FALLESEN  
ROBERT E. STAUFFER  
INVENTORS

Newton M. Perkins  
BY R. Frank Smith  
ATTORNEYS

## UNITED STATES PATENT OFFICE

2,566,180

DIRECT POSITIVE PHOTOGRAPHIC COLOR  
PROCESS

George Earle Fallesen and Robert Eliot Stauffer,  
Rochester, N. Y., assignors to Eastman Kodak  
Company, Rochester, N. Y., a corporation of  
New Jersey

Application August 13, 1948, Serial No. 44,214

3 Claims. (Cl. 95—88)

1

This invention relates to photography and particularly to a method of making direct positive color photographs.

Fallesen U. S. application Ser. No. 780,405, filed October 17, 1947, now U. S. Patent 2,497,875, granted February 21, 1950, describes a process of making direct positive photographs in which a special type of silver halide emulsion capable of giving an internal latent image is exposed and developed in a photographic developer which is capable of giving aerial fog. Exposure of this emulsion produces an internal latent image and development of the exposed emulsion in a developer which gives aerial fog, develops a positive image in those regions of the emulsion layer which were not exposed. Stauffer U. S. application Ser. No. 780,569, filed October 17, 1947, now U. S. Patent 2,497,817, granted February 21, 1950, describes a method for obtaining increased aerial fog and higher maximum density of the reversal image in the Fallesen process by the addition to the developer of certain compounds such as benzotriazole which are so constituted as to increase the maximum density of the positive image obtained in developing solutions capable of producing aerial fog.

Glass and Richey, as described in their U. S. application Serial No. 780,574, filed October 17, 1947, now U. S. Patent 2,507,154, granted May 9, 1950, found that the aerial fogging developer of Fallesen could be replaced with a developer containing a primary aromatic amino developing agent and an active methylene coupler compound to form positive silver and dye images. In the Glass and Richey process the formation of the dye image is incidental to the formation of the silver image, since not all color couplers produce the reversal obtained with the active methylene coupler compounds. Couplers of the naphtholic or phenolic type are not operative in the Glass and Richey process. Therefore, while yellow and magenta dye images can be obtained in the Glass and Richey process cyan images have not been obtained and the process has limited utility in the field of color photography.

Ives described, in U. S. application Serial No. 780,318, filed October 17, 1947, now Patent No. 2,533,463, a two-bath method of obtaining direct positive images which permitted a considerably shortened processing time. According to the Ives disclosure, the exposed photographic emulsion was treated for a short time with developer described in the Fallesen, Stauffer or Glass and Richey applications and then followed by treatment with an active black and white developer

capable of developing the surface latent image.

Since the processes described above are not capable of producing a range of colors suitable for natural color photography, it is the primary purpose of our invention to provide a method for the production of natural color images, that is, a method which will permit the formation of direct positive color photographs having a full range of colors.

10 This object is accomplished according to our invention by following a two-bath procedure similar to that of the Ives application Serial No. 780,318, now Patent No. 2,533,463, in which we expose a suitable single layer or multi-layer emulsion to an image, treat the exposed material for a short time in a developer capable of producing surface latent image in the unexposed regions and then treat the exposed material in a developing solution containing a primary aromatic amino developer. To produce a color image, there must be a color coupler either in the developer or in the emulsion layer and either method can be used according to our invention.

15 In the accompanying drawing, sectional views 25 of a photographic element at successive stages in our process are shown.

The photographic emulsion used in the process of our invention is a gelatino-silver halide emulsion such as silver bromide, silver bromo-iodide or silver chloroiodide emulsion. It need not contain optical sensitizing dyes although certain sensitizing dyes may be added to it for the purpose of inducing aerial fog, as well as for optical sensitizing. The emulsion should be undigested or if digested, the digestion should be carried out without the use of surface sensitizers. An emulsion of this type is known as Burton's Emulsion described in Wall "Photographic Emulsions," 1927, pages 52 and 53. A further type of emulsion suitable for our process is an internal latent image emulsion described in Davey and Knott U. S. application Ser. No. 790,232, filed December 6, 1947, now abandoned, of which application Serial No. 82,914, filed 35 March 22, 1949, is a continuation-in-part.

40 Most of the "internal latent image" emulsions are silver bromoiodide of high iodide content, preferably containing at least 10 to 20% of the amount of silver halide as the iodide. Burton's Emulsion is an emulsion of this type having a silver iodide content of approximately 40% of the content of silver halide. It is not absolutely essential, however, for the emulsion to contain silver iodide.

45 55 An "internal latent image" type of silver hal-

ide emulsion may be defined as one which, when a test portion is exposed to a light intensity scale for a fixed time between  $\frac{1}{100}$  and 1 second and developed for 4 minutes at 20° C. in the ordinary "surface" developer (Example 1), exhibits a maximum density not greater than  $\frac{1}{6}$  the maximum density obtained when the same emulsion is equally exposed and developed for 3 minutes at 20° C. in an "internal" type developer (Example 2). Preferably the maximum density obtained with the "surface" developer is not greater than  $\frac{1}{8}$  the maximum density obtained when the same emulsion is developed in the "internal" type developer. Stated conversely, an "internal latent image" emulsion, when developed in an "internal type developer" (Example 2) exhibits a maximum density at least 5 and preferably at least 10 times the maximum density obtained when the emulsion is exposed in the same way and developed in a "surface" developer (Example 1).

According to our method of producing direct positive color images, an emulsion of the type described above is exposed to light rays or to a suitable image and is then bathed for approximately 15 seconds to 1 minute in a selectively fogging developer such as those described in Fallesen U. S. Patent 2,497,875, Stauffer U. S. Patent 2,497,817 or Glass and Richey U. S. Patent 2,507,154. After a brief rinse, the film is placed in an active developer containing a primary aromatic amino developing agent and a color coupler, unless the color coupler is present in the emulsion layer. Color couplers of the proper constitution can be introduced into the emulsion layers either in the form of coupler-solvent dispersions as described in Mannes and Godowsky U. S. Patent 2,304,940 or Jelleay and Vittum U. S. 2,322,027 or as non-wandering couplers of the type described in Fischer U. S. Patent 1,102,028. About ten minutes are generally required to produce the color image, although a shorter time may be sufficient. If the film is allowed to remain in the selectively fogging developer for about 12 to 15 minutes, a positive silver image will be formed. On the other hand, if the film is placed in the color developing solution without being placed in the fogging developing solution, a negative dye image will be produced in some cases and a positive dye image in others. If the color couplers used in the developer are of the type described in Glass and Richey U. S. Patent 2,507,154, a positive dye image will be produced and if the couplers are of the phenolic or naphtholic type, a negative dye image will be produced.

In the short treatment in the selective fogging developer used in our invention, no visible image appears in the emulsion. The treatment is mainly one of preparation and conditioning for subsequent development. Presumably the selectively fogging developer creates development centers on the surface of the silver halide grains and these are more susceptible to development in the active surface type developer used in the second step, than the development centers created inside the grains by the action of the earlier light exposure. When the emulsion is subjected to treatment in the selectively fogging developer, the grains affected by the light exposure are less susceptible to development in the active surface type developer used in the second step, than the development centers created inside the grains by the action of earlier light exposure. When the emulsion is subjected to

treatment in the selectively fogging developer, the grains affected by the light exposure are not susceptible to fogging and therefore do not develop when the emulsion is placed in the active developer.

The results of the various steps in our process will be readily understood by reference to the accompanying drawing which shows in sectional view a film at various stages in the process. As shown in the first stage of Fig. 1 of the drawing, a sensitive element comprising a support 10 having thereon a sensitive emulsion layer 11 of the internal latent image type is exposed to light under an image represented as having a transparent portion 12 and an opaque portion 13. This exposure produces an internal latent image at 14 in the emulsion layer 11.

Treatment of the exposed element in the selectively fogging developer produces a surface latent image at 15 in the portions of the layers which were not exposed without affecting the internal latent image at 14 as shown in the second stage of the drawing.

A treatment of the element in an active color developer reduces the surface latent image to a metallic silver and dye image 16 as shown in the third stage of the drawing. The remaining silver halide and metallic silver are then removed to leave the dye image 17 in the portions of the layer which were unexposed by the original exposure as shown in the final stage of Fig. 1 of the drawing.

Fig. 2 of the drawing illustrates a multi-layer material having a support 18 with superposed emulsion layers 19, 20 and 21 coated thereon. Emulsion layer 19 is a red-sensitive internal latent image emulsion containing a color coupler capable of forming a cyan dye image. Emulsion layer 20 is a green-sensitive internal latent image emulsion containing color coupler capable of producing a magenta dye image. Emulsion layer 21 is a blue-sensitive internal latent image emulsion containing a color coupler capable of producing a yellow dye image. The usual yellow filter layer 22 is present between emulsion layers 20 and 21 to prevent blue light from exposing emulsion layers 19 and 20.

An ordinary "surface type" developer, that is, one which develops an image only on the surface of the grains of an "internal latent image" emulsion is the following.

#### Example 1

55 p-Hydroxyphenylglycine \_\_\_\_\_ grams 10  
55 Sodium carbonate, (crystals) \_\_\_\_\_ do 100  
55 Water to \_\_\_\_\_ liter 1  
55 Development time, 4 min. at 20° C.

An "internal type" developer, that is, one which develops an image inside the grains of an "internal latent image emulsion" is the following:

#### Example 2

65 Hydroquinone \_\_\_\_\_ grams 15  
65 Monomethyl-p-aminophenol sulfate \_\_\_\_\_ do 15  
65 Sodium sulfite (anhdyd.) \_\_\_\_\_ do 50  
65 Potassium bromide \_\_\_\_\_ do 10  
65 Sodium hydroxide \_\_\_\_\_ do 25  
65 Sodium thiosulfate (crystals) \_\_\_\_\_ do 20  
70 Water to \_\_\_\_\_ liter 1  
70 Development time, 3 min. at 20° C.

A developer which produces a direct positive image on exposure and development of an internal latent image emulsion as described in

Stauffer U. S. application Ser. No. 780,569 is the following:

*Example 3*

|                         |       |      |
|-------------------------|-------|------|
| Hydroquinone            | grams | 10.0 |
| Sodium sulfite (des.)   | do    | 16.0 |
| Paraformaldehyde        | do    | 4.0  |
| Sodium carbonate (des.) | do    | 25.0 |
| Benzotriazole           | do    | 0.4  |
| Water to                | liter | 1    |

Active color developers which may be used to produce the positive dye image according to our invention after treatment of the exposed emulsion in a selectively fogging developer are as follows:

*Example 4*

|                            |       |    |
|----------------------------|-------|----|
| p-Amino diethylaniline HCl | grams | 2  |
| Sodium sulfite (des.)      | do    | 2  |
| Sodium carbonate (anhyd.)  | do    | 20 |
| 2,4-dichloro-1-naphthol    | do    | 3  |
| Sodium hydroxide           | do    | 3  |
| Water to                   | liter | 1  |

*Example 5*

|                                |       |    |
|--------------------------------|-------|----|
| p-Amino diethylaniline HCl     | grams | 2  |
| Sodium sulfite (des.)          | do    | 2  |
| Sodium carbonate (anhyd.)      | do    | 20 |
| Acetoacet-2,5-dichloro anilide | do    | 3  |
| Sodium hydroxide               | do    | 3  |
| Water to                       | liter | 1  |

*Example 6*

|                            |       |    |
|----------------------------|-------|----|
| p-Amino diethylaniline HCl | grams | 2  |
| Sodium sulfite (des.)      | do    | 2  |
| Sodium carbonate (anhyd.)  | do    | 20 |
| p-Nitrophenyl acetonitrile | do    | 3  |
| Sodium hydroxide           | do    | 3  |
| Water to                   | liter | 1  |

In place of the couplers described above, any of the customary color-forming compounds may be used.

Our invention will now be described by reference to the following specific example.

An emulsion such as that described in Davey and Knott U. S. application 790,232 was coated on a support, dried and exposed on an Eastman IIb Sensitometer (Jour. Soc. Motion Picture Engineers, vol. 17, 1931, page 536). The exposed film was bathed for 15 seconds at 68° F. in the developer of Example 3 in a shallow tray and after a 5-second rinse in running water was placed immediately in a tank containing one of the developers of Examples 4, 5 and 6 for a period of 10 minutes at 68° F. The three developers produced, respectively, silver and cyan, silver and yellow, and silver and magenta dye images. The silver images were then bleached in the usual way and the undeveloped silver salts fixed out to leave dye images in the gelatin.

To prepare a multi-layer natural color dye image, a support was coated with successive layers of red-sensitive emulsion, green-sensitive emulsion, yellow filter and blue-sensitive emulsion, all emulsions being of the type described in Davey and Knott U. S. application 790,232. The red-sensitive emulsion contained 5-(p-aminophenoxy benzene sulfonamino-1-naphthol), the green-sensitive contained 2-cyano-acetyl-5-(p-sec. amyl benzoylamino) coumarone and the blue-sensitive contained N-amyl-p-benzoyl acetamino benzene sulfonate. All couplers were dispersed in the emulsions as described in Jelley and Vittum U. S. Patent 2,322,027, granted June 15, 1943.

The emulsions were exposed to a step tablet

and were then developed for 15 minutes in the following developer (Example 7):

*Example 7*

|                           |                            |       |   |
|---------------------------|----------------------------|-------|---|
| 5                         | p-Amino diethylaniline HCl | grams | 2 |
| Sodium sulfite (des.)     | do                         | 2     |   |
| Sodium carbonate (anhyd.) | do                         | 20    |   |
| Acetonyl acetone          | do                         | 3     |   |
| Sodium hydroxide          | do                         | 3     |   |
| Water to                  | liter                      | 1     |   |

Cyan, magenta, and yellow dye images were produced in the red-sensitive, green-sensitive and blue-sensitive layers, respectively, and the silver was then converted to a soluble salt and removed by fixing in the usual way.

It will be understood that the modifications included herein are illustrative only and that variations may be made in our process within the scope of the appended claims.

We claim:

1. The method of obtaining a direct positive dye image in a silver halide emulsion layer, which comprises exposing to light rays to which the emulsion is sensitive, a silver halide emulsion layer a test portion of which upon exposure to a light intensity scale for a fixed time between 1/100 and 1 second and development for 3 minutes at 20° C. in the following internal type developer:

|                                  |                  |       |    |
|----------------------------------|------------------|-------|----|
| 30                               | Hydroquinone     | grams | 15 |
| Monomethyl-p-aminophenol sulfate | do               | 15    |    |
| Anhydrous sodium sulfite         | do               | 50    |    |
| Potassium bromide                | do               | 10    |    |
| 35                               | Sodium hydroxide | do    | 25 |
| Sodium thiosulfate               | do               | 20    |    |
| Water to                         | liter            | 1     |    |

gives a maximum density at least 5 times the maximum density obtained when the equally exposed silver halide emulsion is developed for 4 minutes at 20° C. in the following surface developer (I):

|                             |                        |       |    |
|-----------------------------|------------------------|-------|----|
| 45                          | p-Hydroxyphenylglycine | grams | 10 |
| Sodium carbonate (crystals) | do                     | 100   |    |
| Water to                    | liter                  | 1     |    |

50 immersing the exposed emulsion layer in an aerial fogging developer for about 15 seconds to 1 minute, during which time no visible image is formed, then immersing said layer in an active surface-type developer containing a primary aromatic amino developing agent and a color coupler, for approximately 10 minutes during which time a positive dye image is formed in said layer.

55 2. The method of obtaining a direct positive dye image in a silver halide emulsion layer, which comprises exposing to light rays to which the emulsion is sensitive, a silver halide emulsion layer a test portion of which upon exposure to a light intensity scale for a fixed time between 1/100 and 1 second and development for 3 minutes at 20° C. in the following internal type developer:

|                                  |                    |       |    |
|----------------------------------|--------------------|-------|----|
| 65                               | Hydroquinone       | grams | 15 |
| Monomethyl-p-aminophenol sulfate | do                 | 15    |    |
| Anhydrous sodium sulfite         | do                 | 50    |    |
| Potassium bromide                | do                 | 10    |    |
| Sodium hydroxide                 | do                 | 25    |    |
| 70                               | Sodium thiosulfate | do    | 20 |
| Water to                         | liter              | 1     |    |

gives a maximum density at least 5 times the maximum density obtained when the equally exposed silver halide emulsion is developed for 4

minutes at 20° C. in the following surface developer (I):

p-Hydroxyphenylglycine----- grams 10  
Sodium carbonate (crystals)----- do 100  
Water to----- liter 1

immersing the exposed layer in an aerial fogging developer of the following composition for about 15 seconds at 68° F.:

Hydroquinone----- grams 10  
Sodium sulfite (des.)----- do 16  
p-Formaldehyde----- do 4  
Sodium carbonate (anhyd.)----- do 25  
Benzotriazole----- do 0.4  
Water to----- liter 1

then immersing said layer in an active surface-type developer containing a primary aromatic amino developing agent and a color coupler, for approximately 10 minutes during which time a positive dye image is formed in said layer.

3. The method of obtaining a direct positive dye image in a silver halide emulsion layer, which comprises exposing to light rays to which the emulsion is sensitive, a silver halide emulsion layer a test portion of which upon exposure to a light intensity scale for a fixed time between 1/100 and 1 second and development for 3 minutes at 20° C. in the following internal type developer:

Hydroquinone----- grams 15  
Monomethyl-p-aminophenol sulfate----- do 15  
Anhydrous sodium sulfite----- do 50  
Potassium bromide----- do 10  
Sodium hydroxide----- do 25  
Sodium thiosulfate----- do 20  
Water to----- liter 1

gives a maximum density at least 5 times the

maximum density obtained when the equally exposed silver halide emulsion is developed for 4 minutes at 20° C. in the following surface developer (I):

p-Hydroxyphenylglycine----- grams 10  
Sodium carbonate (crystals)----- do 100  
Water to----- liter 1

immersing the exposed layer in an aerial fogging developer of the following composition for about 15 seconds at 68° F.:

Hydroquinone----- grams 10  
Sodium sulfite (des.)----- do 16  
p-Formaldehyde----- do 4  
Sodium carbonate (anhyd.)----- do 25  
Benzotriazole----- do 0.4  
Water to----- liter 1

then immediately immersing said layer in the following active developer for about 10 minutes at 68° F.:

p-Amino-diethylaniline HCl----- grams 2  
Sodium sulfite (des.)----- do 2  
Sodium carbonate (anhyd.)----- do 20  
p-Nitrophenyl acetonitrile----- do 3  
Sodium hydroxide----- do 3  
Water to----- liter 1

thereby forming a positive magenta dye image in said layer.

30 GEORGE EARLE FALLESEN.  
ROBERT ELIOT STAUFFER.

#### REFERENCES CITED

35 The following references are of record in the file of this patent:

Wall: "Photographic Emulsions," publ. 1929 by Amer. Phot. Publ. Co., Boston; pages 52 and 53.